# EUROPEAN PATENT APPLICATION

(11) **EP 0 474 136 A1**
(43) Date of publication of application: **11.03.1992**
(21) Application number: 91114651.2
(22) Date of filing: 30.08.1991
(51) Int. Cl.: G03C 7/30

(54) **Silver halide color photographic material**

(30) Priority: 04.09.1990 JP 234021/90
(71) Applicant: KONICA CORPORATION, Tokyo 160 (JP)
(72) Inventor: Ikeda, Hiroshi, Hino-shi, Tokyo 191 (JP); Suzuki, Katsutoyo, Hino-shi, Tokyo 191 (JP); Ezaki, Atsuo, Hino-shi, Tokyo 191 (JP)
(74) Representative: Henkel, Feiler, Hänzel & Partner

(57) **Abstract**

The improved silver halide color photographic material has a red-sensitive, a green-sensitive and a blue-sensitive silver halide emulsion layer on a support and is characterized in that each of the red-sensitive and green-sensitive silver halide emulsion layers has a three-layer structure in which a low-speed, a medium-speed and a high-speed silver halide emulsion layer are successively coated on the support, with the low-speed silver halide emulsion layer being the closest to the support, the sum of the silver amount in the red-sensitive silver halide emulsion layer being not more than the sum of the silver amount in the green-sensitive silver halide emulsion layer, and the green-sensitive silver halide emulsion layer having the smallest silver amount in the medium-sensitivity silver halide emulsion layer. This photographic material achieves faithful color reproduction, produces a wide latitude in the intense exposure range, and features good process stability.

## Description

### BACKGROUND OF THE INVENTION

This invention relates to a silver halide color photographic material capable of faithful color reproduction. More particularly, this invention relates to a silver halide color photographic material that has a wide latitude in the intense exposure range and that can be processed in a consistent manner.

Silver halide color photographic materials (hereunder sometimes referred to as "color photographic materials"), especially picture-taking color photographic materials, have heretofore been required to satisfy various performance conditions, such as high speed, good image quality, faithful color reproduction and a wide latitude of exposure. On the other hand, many "mini-labs" or "compact labs" are in operation these days in order to shorten the time of processing picture-taking color photographic materials and to reduce the pickup and delivery costs. In such small-scale laboratories, the processing scheme is highly simplified so that the control of processing solutions is often insufficient compared to large-scale laboratories. Therefore, in spite of the marked improvements in hardware and processing agents, the consistency of photographic processing is not necessarily satisfactory in mini-labs or compact labs. Under these circumstances, there is an increasing demand for picture-taking color photographic materials that are improved not only in image quality but also in process stability.

Several methods have been proposed for improving the processability of picture-taking color photographic materials. Among those proposals is allowing individual emulsion layers to be developed at the same speed by properly adjusting the size of silver halide grains or their relative contents of halogens (I, Br and CI). However, this approach has not proved to be completely satisfactory since it imposes substantial limits on granularity, sensitivity and color reproduction. If each of the red- , green- and blue-sensitive layers adopts a single-layer structure, the occurrence of waviness in the characteristic curve can be avoided but then disadvantages result in terms of sensitivity and granularity, so this approach has been difficult to adopt in commercial operations.

Under these circumstances, the present inventors conducted intensive studies in order to obtain a color photographic material that produces high image quality and which yet can be processed in a more consistent way. As a result, the present inventors found that it would be effective to control the silver amount not only in a red-sensitive silver halide emulsion layer but also in a green-sensitive silver halide emulsion layer.

### SUMMARY OF THE INVENTION

An object, therefore, of the present invention is to provide a silver halide color photographic material that has a sufficiently great interimage effect to produce a wider latitude in the intense exposure range.

Another object of the present invention is to provide a silver halide color photographic material that has better process stability.

These objects of the present invention can be attained by a silver halide color photographic material which comprises a red-sensitive, a green-sensitive and a blue-sensitive silver halide emulsion layer on a support, which photographic material is characterized in that each of the red-sensitive and green-sensitive silver halide emulsion layers has a three-layer structure in which a low-speed, a medium-speed and a high-speed silver halide emulsion layer are being provided in this order with respect to the support, the sum of the silver amount in the red-sensitive silver halide emulsion layer being not more than the sum of the silver amount in the green-sensitive silver halide emulsion layer, and the green-sensitive silver halide emulsion layer having the smallest silver amount in the medium-speed silver halide emulsion layer.

### DETAILED DESCRIPTION OF THE PREFERRED EMBODIMENT

The present invention is described below in greater detail.

The silver halide color photographic material of the present invention has a red-sensitive, a green-sensitive and a blue-sensitive silver halide emulsion layer on a base and is characterized in that each of the red-sensitive and green-sensitive silver halide emulsion layers has a three-layer structure in which a low-speed, a medium-speed and a high-speed silver halide emulsion layer are successively coated on the support, with the low-speed silver halide emulsion layer being the closest to the support, that the sum of the silver amount in the red-sensitive silver halide emulsion layer is not more than the sum of the silver amount in the green-sensitive silver halide emulsion layer, and that the green-sensitive silver halide emulsion layer has the smallest silver amount in the medium-speed silver halide emulsion layer.

Preferably, the blue-sensitive silver halide emulsion layer also has a three-layer structure in which a low-speed, a medium-speed and a high-speed silver halide emulsion layer are successively coated on the support, with the low-speed silver halide emulsion layer being the closest to the support.

The silver halide color photographic material of the present invention preferably has a total silver amount of 15 - 120 mg/dm², more preferably 35 - 85 mg/dm².

The amount of silver in each of the red-sensitive and green-sensitive silver halide emulsion layers in the color photographic material of the present invention may be set to any desired value as long as the sum of the silver amount of light-sensitive silver halides in the red-sensitive silver halide emulsion layer is not more than the sum of the silver amount of light-sensitive silver halides in the green-sensitive silver halide emulsion layer. Preferably, the ratio of the sum of the silver amount in the red-sensitive silver halide emulsion layer to the sum of the silver amount in the green-sensitive silver halide emulsion layer is in the range of 0.6 - 1.0, more preferably in the range of 0.8 - 0.95.

The amounts of silver in the low-speed, medium-speed and high-speed silver halide emulsion layers that make up the green-sensitive emulsion layer of the color photographic material of the present invention may be set to any desired proportions as long as the medium-speed silver halide emulsion layers has the smallest silver deposit. Preferably, the amount of silver increases in the order of the medium-speed, low-speed and high-speed silver halide emulsion layers.

The color photographic material of the present invention preferably contains a DIR compound. The term "DIR compound" as used herein means a compound that, upon reaction with the oxidation product of a color developing agent, releases a development inhibitor or a compound capable of releasing an inhibitor.

If a DIR compound is to be used in the present invention, it is preferably diffusible DIR compound. A diffusible DIR compound is such a compound that a development inhibitor or a compound capable of releasing an inhibitor that are released upon reaction with the oxidation product of a color developing agent has a diffusibility of at least 0.34, preferably at least 0.40, as measured by the method of evaluation to be just described below.

The method of diffusibility evaluation as applicable to the present invention comprises the following steps.

First, two samples of light-sensitive material (I) and (II) are prepared by coating the following layers on a transparent base.

### Sample (I): sample having a green-sensitive silver halide emulsion layer, which is prepared by the following procedure

A gelatin based coating solution that contains silver iodobromide (6 mol% Agl; average grain size, 0.48 am) spectrally sensitized to green light and that also contains a coupler (for its structure, see below) in an amount of 0.07 mole per mole of silver is coated on the base to give 1.1 g/m² of silver and 3.0 g/m²0f gelatin; subsequently, a gelatin based coating solution that contains neither chemically nor spectrally sensitized silver iodobromide (2 mol% Agl; average grain size, 0.08 am) is coated to give 0.1 g/m² of silver and 0.8 g/m² of gelatin, whereby a protective layer is formed.

### Sample (II): same as sample (I) except that silver iodobromide is absent from the protective layer

In both samples, a gelatin hardener and a surfactant are also contained in the individual layers.

After exposure to white light through an optical wedge, each of samples (I) and (II) is processed by the following scheme using two kinds of developing solution, one incorporating various development inhibitors in an amount that suppresses the sensitivity of sample (II) by 60% (ΔlogE = 0.22 as expressed on a logarithm scale) and the other incorporating no such development inhibitors.

The processing solutions used in this processing scheme have the following formulas:

### Bleaching solution

Fixing solution

If So and So are respectively written for the sensitivities of samples (I) and (II) in the absence of a development inhibitor and if Sₗ and Sₗₗ are respectively written for the sensitivities of samples (I) and (II) in the presence of a development inhibitor, then the following relations hold:
Desensitization of sample (I): AS = So - Sₗ
Desensitization of sample (II): ΔSₒ = Sₒ' - Sₗₗ
Diffusibility = ΔS/ΔSₒ.

In the above disscussion, all sensitivity values are expressed as -logE, or the logarithm of the reciprocal of the exposure necessary to provide a density of fog + 0.3.

The diffusibility data obtained for several development inhibitors by the above-described method are shown in the following table.

It is preferred for the purposes of the present invention to use DIR compounds that release groups having diffusibility values within the range set forth above but any other DIR compounds may of course be used.

Compounds of the type described above which may advantageously be used in the present invention typically have the following general structural formula: where A is a coupler residue; m is 1 or 2; Y is a development inhibitor group or a group capable of releasing a development inhibitor that are bound to the coupler residue A at the coupling site and that are released upon reaction with the oxidation product of a color developing agent, said group Y having a diffusibility of at least 0.40.

In the general formula (D-1), Y is typically represented by any one of the following general formulas (D-2) to (D-19).

In general formulas (D-2) to (D-7), Rd₁ represents a hydrogen atom, a halogen atom, or a group selected from among the following: alkyl, alkoxy, acylamino, alkoxycarbonyl, thiazolylideneamino, aryloxycarbonyl, acyloxy, carbamoyl, N-alkylcarbamoyl, N,N-dialkylcarbamoyl, nitro, amino, N-arylcarbamoyloxy, sulfamoyl, N-alkylcarbamoyloxy, hydroxy, alkoxycarbonylamino, alkylthio, arylthio, aryl, hetero ring, cyano, alkylsulfonyl and aryloxycarbonylamino; n represents 0, 1 or 2, provided that when n is 2, Rd₁ s may be the same or different.

The total number of carbon atoms in n Rd₁ s is from 0 to 10. The number of Rd₁ s in the general formula (D-6) is from 0 to 15.

In the general formula (D-6), X represents an oxygen or sulfur atom.

In the general formula (D-8), Rd₂ represents an alkyl group, an aryl group or a hetero ring.

In the general formula (D-9), Rd₃ represents a hydrogen atom or a group selected selected from among alkyl, cycloalkyl, aryl and a hetero ring; Rd₄ represents a hydrogen atom, a halogen atom or a group selected from among alkyl, cycloalkyl, aryl, acylamino, alkoxycarbonylamino, aryloxycarbonylamino, alkanesulfonamido, cyano, hetero ring, alkylthio and amino.

When Rd,, Rd₂, Rd₃ or Rd₄ represents an alkyl group, it may optionally contain a substituent and it may be straight- chained or branched.

When Rd₁, Rd₂, Rd₃ or Rd₄ represents an aryl group, it may optionally contain a substituent.

When Rd₁, Rd₂, Rd₃ or Rd₄ represents a hetero ring, it may optionally contain a substituent and is preferably a single or condensed 5- or 6-membered ring that contain at least one hetero atom selected from among a nitrogen atom, an oxygen atom and a sulfur atom; examples of the preferred hetero ring include pyridyl, quinolyl, furyl, benzothiazolyl, oxazolyl, imidazolyl, thiazolyl, triazolyl, benzotriazolyl, imido and oxazine.

In general formulas (D-6) and (D-8), Rd₂ contains 0 - 15 carbon atoms.

In general formula (D-9), Rd₃ and Rd₄ contain a total of 0 - 15 carbon atoms. where TIME is a group that binds to A at the coupling site and that can be cleaved upon reaction with the oxidation product of a color developing agent; after cleavage from the coupler, TIME is capable of releasing the group INHIBIT at a properly controlled rate; upon such release, the group INHIBIT becomes a development inhibitor [examples of the group INHIBIT are those which are represented by general formulas (D-2) to (D-9)].

In general formula (D-10), -TIME-INHIBIT is typically represented by the following general formulas (D-11) to (D-19):

In general formulas (D-11) to (D-15) and (D-18), Rd₅ represents a hydrogen atom, a halogen atom, or a group selected from the following: alkyl, cycloalkyl, alkenyl, aralkyl, alkoxy, alkoxycarbonyl, anilino, acylamino, ureido, cyano, nitro, sulfonamido, sulfamoyl, carbamoyl, aryl, carboxy, sulfo, hydroxy or alkanesulfonyl. In general formulas (D-11) to (D-13), (D-15) and (D-18), Rd₅s may combine together to form a condensed ring; in general formulas (D-11), (D-14), (D-15) and (D-19), Rd₆ representsan alkyl group, an alkenyl group, an aralkyl group, a cycloalkylgroup, a hetero ring or an aryl group; in general formulas (D-16) and (D-17), Rd₇ represents a hydrogen atom or a group selected from among alkyl, alkenyl, aralkyl, cycloalkyl, hetero ring and aryl; in general formula (D-19), Rd₈ and Rdₛ each represents a hydrogen atom or an alkyl group (preferably a C₁₋₄ alkyl group); in general formulas (D-11) and (D-15) to (D-18), k represents an integer of 0, 1 or 2; in general formulas (D-11) to (D-13), (D-15) and (D-18), 1 represents an integer of 1 - 4; in general formula (D-16), m represents an integer of 1 or 2, provided that when m is 2, Rd₇s may be the same or different; in general formula (D-19), n represents an integer of 2 - 4, provided that n Rd₈s and Rdss may be the same or different; in general formulas (D-16) to (D-18), B represents an oxygen atom or (where Rd₆ has the same meaning as already defined); in general formula (D-16), represents either a single bond or a double bond and in the case of a single bond, m is 2 and, in the case of a double bond, m is 1. The group INHIBIT is the same as defined by general formulas (D-2) to (D-9) except for the number of carbon atoms.

In the group INHIBIT, the total number of carbon atoms in Rd₁ in one molecule of general formulas (D-2) to (D-7) is from 0 to 32; the number of carbon atoms in Rd₂ in general formula (D-8) is from 1 to 32; and Rd₃ and Rd₄ in general formula (D-9) contains a total of 0 - 32 carbon atoms.

When Rd₅, Rd₆ and Rd₇ each represents an alkyl group, an aryl group or a cycloalkyl group, they may optionally contain a substituent.

Preferred diffusible DIR compounds are those which are represented by general formula (D-2), (D-3) or (D-10) and in the case of a diffusible DIR compound represented by (D-10), INHIBIT is preferably represented by general formula (D-2), (D-6) (the case where X in (D-6) is an oxygen atom is particularly preferred) or (D-8) (the case where Rd₂ in (D-8) is a hydroxyaryl or a C₁ -₅ alkyl is particularly preferred).

The coupler component represented by A in general formula (D-1) may be exemplified by a yelow dye image forming coupler residue, a magenta dye image forming coupler residue, a cyan dye image forming coupler residue and a colorless coupler residue.

The diffusible DIR compounds that are preferably used in the present invention may be exemplified by, but not limited to, the following compounds:
Exemplary diffusible DIR compounds

### Definitions of R₁, R₂ and Y

These and other examples of the diffusible DIR compounds that can be used in the present invention are described in U.S. Patent Nos. 4,234,678, 3,227,554, 3,617,291, 3,958,993, 4,149,886, 3,933,500, Unexamined Published Japanese Patent Application Nos. 56837/1982 and 13239/1976, U.S. Patent Nos. 2,072,363 and 2,070,266, and Research Disclosure No. 21228, December 1981.

In the light-sensitive material of the present invention, diffusible DIR compounds are preferably used in amounts of 0.0001 - 0.1 mol per mole of silver halide, with the range of 0.001 - 0.05 mole being particularly preferred.

It is generally preferred that the silver halide emulsions in the light-sensitive material of the present invention are such that, after physical and chemical ripening, they have been subjected to spectral sensitization in accordance with the color forming light-sensitive layers to be used. Illustrative additives that can be used in such steps are described in Research Disclosure Nos. 17643, 18716 and 308119 (which are respectively abbreviated as RD 17643, RD 18716 and RD 308119). Useful additives are given below together with the relevant portions of description in those three issues of Research Disclosure:

Examples of the known photographic additives that may be used in the practice of the present invention are also described in the three issues of Research Disclosure, as shown below:

Various couplers can be used in the light-sensitive material of the present invention depending upon the color to be formed in each of the color-sensitive layers. Specific examples of useful couplers are given below together with the relevant portions of description in two issues of Research Disclosure.

When various additives are used in the light-sensitive material of the present invention, they may be incorporated by any suitable method such as the dispersion method described in RD 308119 under item XIV.

In the present invention, supports of the types described on page 28 of RD 17643, pages 647-648 of RD 18716 and under item XVII of RD 308119.

The light-sensitive material of the present invention may use a filter layer, an intermediate layer and other auxiliary layers of the types described under item VII-K of RD 308119, supra.

The light-sensitive material of the present invention may adopt a conventional layer order, an inverse layer order, a unit structure and other layer orders of the types described under item VII-K of RD 308119, supra.

The light-sensitive material of the present invention may be applicable to various color photographic materials as typified by color negative films for general use or motion pictures, color reversal films for slides or TV, color paper, color positive films and color reversal paper.

The light-sensitive material of the present invention may be developed by conventional methods of the types described on pages 28-29 or RD 17643, on page 615 of RD 18716, and under item XIX or RD 308119.

The following examples are provided for the purpose of further illustrating the present invention but are in no way to be taken as limiting.

Unless otherwise noted, the amounts of addition of components to silver halide photographic materials are expressed in grams per square meter. The amounts of silver halides and colloidal silver are expressed in terms of silver.

### Example 1

Fifteen layers having the formulas described below were successively coated on a triacetyl cellulose film support, with the first layer being the closest to the base, whereby a sample of multi-layered color photographic material designated sample 1 was prepared.

### Sample 1 :

First layer: Anti-halation layer (HC-1)

### Second layer: Intermediate layer (IL-1)

### Gelatin 1.3

Third layer: Less red-sensitive emulsion layer (RL)

Fourth layer: Medium red-sensitive emulsion layer (RM)

Fifth layer: Highly red-sensitive emulsion layer (RH)

Sixth layer: Intermediate layer (IL-2)

### Gelatin 0.8

Seventh layer: Less green-sensitive emulsion layer (GL)

Eighth layer: Medium green-sensitive emulsion layer (GM)

Ninth layer: Highly green-sensitive emulsion layer (GH)

Tenth layer: Yellow filter layer (YC)

Eleventh layer: Intermediate layer

Twelfth layer: Less blue-sensitive emulsion layer (BL)

Thirteenth layer: Highly blue-sensitive emulsion layer (BH)

Fourteenth layer: First protective layer (Pro-1)

Fifteenth layer: Second protective layer (Pro-2)

Sample 101 also contained a coating aid Su-1, a dispersion aid Su-2, a viscosity modifier, hardeners H-1 and H-2, a stabilizer ST-1, an antifoggant AF-1, and two kinds of antifoggant AF-2 having Mw of 10,000 and 1,100,000.

Additional samples 2 - 15 were prepared in the same way except that the red-sensitive silver halide emulsion layers (layers 3 - 5), or green-sensitive silver halide emulsion layers (layers 7 - 9), or blue-sensitive silver halide emulsion layers (layers 12 and 13) were modified as follows.

Sample 2 (comparison):
Third layer: same as in sample 1
Fourth layer: same as in sample 1
Fifth layer: same as in sample 1
Seventh layer: same as in sample 1
Eighth layer: Medium green-sensitive emulsion layer (GM)

Ninth layer: Highly green-sensitive emulsion layer (GH)

Twelfth layer: same as in sample 1
Thirteenth layer: same as in sample 1

### Sample 3 (comparison):

Third layer: same as in sample 1
Fourth layer: same as in sample 1
Fifth layer: same as in sample 1
Seventh layer: Less green-sensitive emulsion layer (GL)

Eighth layer: Medium green-sensitive emulsion layer (GM)

Ninth layer: Highly green-sensitive emulsion layer (GH)

Twelfth layer: same as in sample 1
Thirteenth layer: same as in sample 1

### Sample 4 (comparison):

Third layer: same as in sample 1
Fourth layer: same as in sample 1
Fifth layer: same as in sample 1

Seventh layer: Less green-sensitive emulsion layer (GL)

Eighth layer: Medium green-sensitive emulsion layer (GM)

Ninth layer: Highly green-sensitive emulsion layer (GH)

Twelfth layer: same as in sample 1
Thirteenth layer: same as in sample 1

### Sample 5 (comparison):

Third layer: same as in sample 1
Fourth layer: same as in sample 1
Fifth layer: same as in sample 1

Seventh layer: Less green-sensitive emulsion layer (GL)

Eighth layer: Medium green-sensitive emulsion layer (GM)

Ninth layer: Highly green-sensitive emulsion layer (GH)

Twelfth layer: same as in sample 1
Thirteenth layer: same as in sample 1

### Sample 6 (comparison):

Third layer: Less red-sensitive emulsion layer (RL)

Fourth layer: Medium red-sensitive emulsion layer (RM)

Fifth layer: Highly red-sensitive emulsion layer (RH)

Seventh layer: same as in sample 1
Eighth layer: same as in sample 1
Ninth layer: same as in sample 1
Twelfth layer: same as in sample 1
Thirteenth layer: same as in sample 1

### Sample 7 (comparison):

Third layer: Less red-sensitive emulsion layer (RL)

Fourth layer: Medium red-sensitive emulsion layer (RM)

Fifth layer: Highly red-sensitive emulsion layer (RH)

Seventh layer: same as in sample 1
Eighth layer: same as in sample 1
Ninth layer: same as in sample 1
Twelfth layer: same as in sample 1
Thirteenth layer: same as in sample 1

### Sample 8 (invention):

Third layer: same as in sample 7
Fourth layer: same as in sample 7
Fifth layer: same as in sample 7
Seventh layer: same as in sample 4
Eighth layer: same as in sample 4
Ninth layer: same as in sample 4
Twelfth layer: same as in sample 1
Thirteenth layer: same as in sample 1

### Sample 9 (invention):

Third layer: Less red-sensitive emulsion layer (RL)

Fourth layer: same as in sample 7
Fifth layer: same as in sample 1
Seventh layer: same as in sample 5
Eighth layer: same as in sample 5
Ninth layer: same as in sample 5
Twelfth layer: same as in sample 1
Thirteenth layer: same as in sample 1

### Sample 10 (invention):

Third layer: Less red-sensitive emulsion layer (RL)

Fourth layer: Medium red-sensitive emulsion layer (RM)

Fifth layer: Highly red-sensitive emulsion layer (RH)

Seventh layer: same as in sample 5
Eighth layer: same as in sample 5
Ninth layer: same as in sample 5
Twelfth layer: same as in sample 1
Thirteenth layer: same as in sample 1

### Sample 11 (invention):

Third layer: same as in sample 7
Fourth layer: same as in sample 7
Fifth layer: same as in sample 7
Seventh layer: same as in sample 5
Eighth layer: same as in sample 5
Ninth layer: same as in sample 5
Twelfth layer: same as in sample 1
Thirteenth layer: same as in sample 1

### Sample 12 (invention):

Third layer: Less red-sensitive emulsion layer (RL)

Fourth layer: Medium red-sensitive emulsion layer (RM)

Fifth layer: Highly red-sensitive emulsion layer (RH)

Seventh layer: same as in sample 5
Eighth layer: same as in sample 5
Ninth layer: same as in sample 5
Twelfth layer: same as in sample 1
Thirteenth layer: same as in sample 1

### Sample 13 (comparison):

Same as sample 1 except that DI-1, DI-2 and DI-3 were absent from layers 3, 4, 5 and 8

### Sample 14 (invention):

Same as sample 8 except that DI-1, DI-2 and DI-3 were absent from layers 3, 4, 5 and 8

### Sample 15 (invention):

First to eleventh layers: same as in sample 10 Twelfth layer: Less blue-sensitive emulsion layer (BL)

Thirteenth layer: Medium blue-sensitive emulsion layer (BM)

Fourteenth layer: Highly blue-sensitive emulsion layer (BH)

Fifteenth layer: same as layer 14 of sample 1
Sixteenth layer: same as layer 15 of sample 1

Emulsions Em-1 to Em-6 which were used in the preparation of samples 1 - 15 were all monodispersed emulsions, as characterized below:
Em-1: silver iodobromide emulsion (average grain size, 0.3 µm; 2 mol% Agl)
Em-2: silver iodobromide emulsion (average grain size, 0.4 µm; 8 mol% Agl)
Em-3: silver iodobromide emulsion (average grain size, 0.7 µm; 8 mol% Agl)
Em-4: silver iodobromide emulsion (average grain size, 0.8 µm; 8 mol% Agl)
Em-5: silver iodobromide emulsion (average grain size, 0.9 µm; 8 mol% Agl)
Em-6: silver iodobromide emulsion (average grain size, 1.0 µm; 10 mol% Agl)

Each of samples 1 - 15 was divided into two groups. One group of samples was given imagewise exposure to white light and the other group was given imagewise exposure to red light through an optical filter (Wratten W-26 of Kodak). Thereafter, all samples were color-processed by the following scheme.

The processing solutions had the following formulas.

### Bleaching solution

### Fixing solution

Stabilizing solution

For each of the processed samples, the magenta and cyan image densities were measured at varying exposures to construct characteristic curves.

Each of samples 1 - 15 was subjected to photographic sensitometry and Si, or the point for minimum cyan density (Dmin) + 0.15, was plotted to determine ΔD_{R-N}, or the difference in density between a sample given imagewise exposure to white light and a sample given imagewise exposure to red light when exposure of S₁ + 1.5 of logE was given.

By photographic sensitometry, Sᵢ, or the point for minimum magenta density (Dmin) + 0.15 was also plotted and ΔD, or the difference in density between a sample given imagewise exposure to white light at S₁ + 2.0 of logE and a sample given imagewise exposure to white light at S₁ + 2.8 of logE, was determined for each of samples 1 - 15.

The results are shown in Table 1.

As one can see from Table 1, the samples prepared in accordance with the present invention had sufficiently great density differences of ΔD_{R-N} to provide high color purity. In addition, they had large density differences of ΔD in the intense exposure range to insure fine details in the highlights of image. It should also be noted that by using diffusible DIR compounds in the samples of the present invention, the differences of ΔD_{R-N} and ΔD could be further increased over the comparative samples.

### Example 2

In order to evaluate the process stability of samples 1 - 15, two other color developing solutions having pHs of 9.90 and 10.3 were also prepared as in Example 1 and each sample was processed with the color developing solutions at three different pHs after imagewise exposure to white light.

For each of the processed samples, the cyan and magenta densities were, measured to construct characteristic curves. The gradient of each characteristic curve was determined for the range of S₁ and S₁ + 1.5 of logE, where S₁ was the point for minimum density (Dmin) + 0.15. Thereafter, γ_{H}/γ_{M} and γ_{L}/γ_{M} were calculated, where γ_{M} was the gradient of characteristic curve at pH = 10.1, γ_{H} was the gradient at pH = 10.3, and γ_{L} was gradient at pH = 9.90.

The results are shown in Table 2 below.

As one can see from Table 2, the samples of the present invention had gamma ratios near to unity and this indicates the high process stability of those samples.

The same results were obtained when the samples were processed under running conditions. The running process was continued until the replenishers were supplied in an amount three times the capacity of the stabilizing tanks.

The stabilizing step was performed in a countercurrent fashion using three tanks, with the last tank being supplied with the replenisher of stabilizing solution while the overflow was admitted into the preceeding tank. The overflow from the first stabilizing tank subsequent to the fixing tank was partly (275 ml/m²) admitted into the last stabilizing tank.

### Formula of the replenisher of color developing solution

Formula of bleaching solution

### Formula of the replenisher of bleaching solution

### Formula of fixing solution and its replenisher

Formula of stabilizing solution and its replenisher

As described on the foregoing pages, the silver halide color photographic material of the present invention achieves a sufficiently great interimage effect and faithful color reproduction to produce a wide latitude in the intense exposure range. In addition, it has good process stability.

## Claims

1. A silver halide color photographic material which comprises a red-sensitive, a green-sensitive and a blue-sensitive silver halide emulsion layer on a support, the improvement wherein each of the red-sensitive and green-sensitive silver halide emulsion layers has a three-layer structure in which a low-speed, a medium-speed and a high-speed silver halide emulsion layer being provided in this order with respect to the support, the sum of the silver amount in the red-sensitive silver halide emulsion layer being not more than the sum of the silver amount in the green-sensitive silver halide emulsion layer, and the green-sensitive silver halide emulsion layer having the smallest silver amount in the medium-speed silver halide emulsion layer.

2. A silver halide color photographic material according to claim 1, wherein the ratio of the sum of the silver amount in the red-sensitive silver halide emulsion layer to the sum of the silver amount in the green-sensitive silver halide emulsion layers is in the range of 0.6 - 1.0.

3. A silver halide color photographic material according to claim 1, wherein the silver amount in the green-sensitive silver halide emulsion layers increase in the order of the medium-speed, low-speed and high-speed silver halide emulsion layers.

4. A silver halide color photographic material according to calim 1, wherein the ratio of the sum of the silver amount in the red-sensitive silver halide emulsion layer to the sum of the silver amount in the green-sensitive silver halide emulsion layers is in the range of 0.8 - 0.95, the silver amount in the green-sensitive silver halide emulsion layers increase in the order of the medium-speed, low-speed and high-speed silver halide emulsion layers, and a DIR compound is incorporated in at least one layer of the silver halide emulsion layers.

5. A silver halide color photographic material according to claim 1, wherein at least one of the light-sensitive silver halide emulsion layers contains a compound of the following general formula (D-1):
A - (Y)m
where A is a coupler residue; m is 1 or 2; Y is a development inhibitor group or a group capable of releasing a development inhibitor that are bound to the coupler residue A at the coupling site and that are released upon reaction with the oxidation product of a color developing agent, said group Y having a diffusibility of at least 0.40.

6. A silver halide color photographic material according to claim 5, wherein Y is represented by either one of the following formulas:
(where X is an oxygen atom or a sulfur atom; and Rd₁ is an alkyl group having 1 - 10 carbon atoms); and
(where Rd₂ is an optionally substituted aryl group).
